

## 1

3,026,170

## MANUFACTURE OF VISCOSE RAYON

Arnold L. McPeters, West Asheville, N.C., assignor to  
American Enka Corporation, Enka, N.C., a corpora-  
tion of Delaware

No Drawing. Filed Nov. 29, 1957, Ser. No. 699,516

4 Claims. (Cl. 18—54)

The present invention relates to the manufacture of rayon yarns, filaments, films and the like and more particularly to the production of high tenacity viscose rayon yarn, that is characterized by its high tenacity which makes it especially suitable for use in reinforcing rubber articles such as cord tires and the like.

Due to extensive research being conducted by various rayon manufacturers in recent times, improvements in the physical properties of rayon have been and are being made. These improvements consist of, for example, increasing the breaking strength and elongation at the break of the thread, increasing wet and dry strengths, lowering of the secondary swelling, and increasing the resistance to flex fatigue, abrasion and soiling. Most of the recent improvements seem to bear relationship with the formation of a thread having skin throughout most or all of its cross-section, which indicates, at least, that the molecular crystallinity of the thread has been changed.

Perhaps, the most important recent development is the use of special additives in the spinning system, preferably in the viscose. The precise theory of how the additives affect the coagulation and regeneration of cellulose in the viscose to produce an improved thread has not been definitely established, with various and different views having been expressed. However, it is known that these additives, now referred to as viscose modifiers in the art, tend to retard the regeneration and contribute to the formation of filaments having a large degree of skin and a cross-section with a relatively smooth uncrenulated surface.

Among the first known viscose modifiers, there were included certain aliphatic monoamines and certain quaternary ammonium compounds as disclosed in U.S. Patents 2,535,044, 2,535,045 and 2,536,014. Other additives having in part or the same effect as the aforesaid amine additives are known.

It is known to employ polymerized alkylene oxides as spinning assistants in the spinbath in extremely small amounts to prevent the clogging of spinneret orifices as disclosed in U.S. Patent 2,442,331. Moreover, it is disclosed in Belgian Patent 547,681 that polyethylene oxide with a medium molecular weight of 300—10,000 when added to the viscose in amounts of 0.5—19% by weight of the cellulose influences the formation of viscose rayon filaments of the skin-type with non-crenulated surfaces and high strength. Also, it is disclosed in U.S. Patent 2,696,423 that the combination of the polyethylene oxide compounds having a molecular weight of from about 300 to 1000, among other ether-type modifiers, may be admixed with certain dithiocarbamate modifiers to increase the modification thereof. It is to be understood that the use of polyalkylene oxide compounds as spinning assistants or as per se a viscose modifier forms no part of the present invention.

There is disclosed in copending application Serial No. 609,792, filed September 14, 1956, and having common ownership herewith, a process for the manufacture of high strength yarn, whereby viscose is spun into a spinbath, the acid content of which is low enough to entail heavy zinc and sulfur containing deposits in and around the spinbath container so that spinning becomes impractical, characterized in that the spinning process is carried out in the presence of a sufficiently large quantity of certain ethoxylated cation-active quaternary ammonium

## 2

compounds to bring about a modification of the regeneration of the cellulose, while simultaneously preventing the formation of the undesirable deposits. These amine additives are called "Ethoquads"; and the yarn so produced has excellent fatigue resistance and remarkable strength values, especially suitable for tire cords.

The "Ethoquad" viscose modifier disclosed in said co-pending application has the following general formula:



where  $R_1$  and  $R_2$  represent preferably an alkyl radical but may include an aryl or alicyclic radical with  $R_1$  preferably being an alkyl radical containing six or more carbon atoms and  $R_2$  being an alkyl radical containing one to three carbon atoms;  $Z$  represents an anion having substantially no surface activity such as hydroxide, halide, sulfate, acetate, etc.;  $x$  and  $y$  are whole numbers of at least one with the preferred combined value of  $x$  and  $y$  being 2 to 50 or more;  $n$  is a whole number, possibly one but preferably two and no more than four.

However, in practice, it was found that for a set of given spinning conditions there existed an optimum concentration above which the use of the "Ethoquad" gave very little or no additional improved modification. Therefore, it was thought that the use of the additives as modifiers had certain limitations.

While the known modifiers are useful and influence, in a favorable manner, the formation of yarn having improved properties, it is desired to obtain further improvement in the properties, such as improved cord strength. It is recognized that the tenacity of viscose rayon yarn considerably diminishes when processed into a cord, for example, a tire cord.

It is an object of the present invention to provide a method for the manufacture of filaments of regenerated cellulose by the viscose process which have improved physical properties in general and which may be twisted and plied into a cord construction with a minimum loss in tenacity.

It is another object of the present invention to provide a viscose spinning composition containing a novel combination of modifiers from which viscose rayon yarn of improved physical properties may be spun.

Other objects and advantages of the present invention will become apparent herein.

In a very surprising manner, it was found that the aforesaid objects are accomplished by spinning viscose that contains a synergistic combination of additives consisting of certain polyethylene oxide compounds and certain ethoxylated cation-active quaternary ammonium compounds in amounts to bring about a modification of the cellulose that results in the production of viscose rayon filaments having improved properties as compared to filaments produced under the influence of either type of additive when employed singularly. The viscose containing the combination of additive is spun according to the viscose process into filaments in an aqueous acidic coagulating bath containing a zinc salt. Thereafter, the filaments are given a high degree of stretch before complete regeneration thereof.

The degree of polymerization of the polyethylene oxide additives may vary depending upon the spinning conditions and the other additives employed. However, the improvement of the present invention is attained only when the molecular weight of the polymerized ethylene oxide lies in the range of about 1500—4500. Below the lower limit the modifying power diminishes; above the

upper limit the additive may not dissolve in the viscose to a required minimum quantity. It has been found that the polyethylene oxide compounds induce the desired modifying effect when added to the viscose in amounts of 0.5-5.0% by weight based on the cellulose content in the viscose, hereinafter referred to in short as (C.I.V.).

In general, the quaternary ammonium compounds contemplated to be incorporated in the viscose with the polyethylene oxide compounds are the so-called "Ethoquads" as described above in detail. More particularly, the viscose modifier for this purpose has the following general formula:



15

where  $\text{R}_1$  is an alkyl radical with at least 6 carbon atoms;  $x+y=2-50$ ; and  $\text{Z}$  is an innocuous anion. The amount of the just described additive should be used in the range of 0.5-5.0% (C.I.V.) in order to obtain the desired optimum modifying effect.

It is essential to the invention that the combination of the polyethylene oxide compounds and the ethoxylated cation-active quaternary ammonium compounds be employed in a minimum total concentration of at least 2.0% (C.I.V.), otherwise, the enhanced modification will not be attained.

The viscose containing the aforesaid combination may have other materials, such as delustrants, incorporated therein and may be prepared in part or in whole from wood pulp, with the degree of maturity and the percentages of cellulose and alkali of the viscose not being especially critical. But better results are obtainable when the viscose contains from 5.5 to 8.0% cellulose and from 4.0 to 6.0% alkali and has a maturity in the range of 10-18 NH<sub>4</sub>Cl number. Generally these variables are correlative with each other, but not strictly so in order to obtain the improved yarn properties of the present invention, depending upon the other spinning constants. The modifiers may be incorporated in the spinning system in a variety of ways, such as by adding the additives during the dissolving operation or by injecting the additives into a stream of viscose being pumped to the spinneret.

The coagulating bath into which this viscose is extruded through a spinneret immersed therein should contain a soluble zinc salt, such as zinc sulfate in the amount of not less than 2%, preferably 3-5% and more. Moreover, the sulfuric acid concentration of the bath may and for better results should be lower than concentrations ordinarily used in viscose rayon production. For example, the amount of acid should be less than 7% with the maintenance of a minimum concentration sufficient to coagulate and partially regenerate the cellulose. Other salts, such as sodium sulfate and spinning assistants are also contained in the spinbath. Preferably, the spinbath should have a temperature of about 40 to 70° C. The length of thread immersion depends upon the spinning speed as well as the particular spinbath employed. Since regeneration is retarded under the spinning conditions described herein, it is preferred to conduct the thread through a spinning tube, of the type described in U.S. Patent No. 2,908,937. As shown therein, the thread is passed through the tube during at least part of its travel in the spinbath.

After being withdrawn from the spinbath in a conventional manner, the freshly spun viscose thread is stretched in the excess of 50%, preferably by 80-100% or higher. To obtain the best results, the stretch is applied in a weakly acidic second bath at a temperature, preferably above 80° C., and best at 95° C. The thread is then taken up in package form and aftertreated, or aftertreated in a continuous fashion and then taken up in package form.

The thread produced in accordance with the present invention is particularly characterized by its very low loss in tenacity when twisted into cord. In addition, the thread has lower secondary swelling, increased resistance to flex fatigue and other improvements which make it especially suitable for use as reinforcing cords in tires, conveyor belts, etc. Furthermore, the thread has the so-called skin structure and non-crenulated surfaces associated with thread produced under the influence of a viscose modifier.

The following examples are illustrative of the practice of the present invention as described herein. All concentrations unless otherwise noted are calculated as percentages by weight based on the viscose or the spinbath.

#### EXAMPLE I

Alkali cellulose was prepared in the conventional manner from wood pulp to obtain the desired degree of polymerization of about 460. This alkali cellulose was xanthated at 25° C. with 36% CS<sub>2</sub> (C.I.V.). The xanthate crumbs so produced were dissolved in a solution of sodium hydroxide of a predetermined alkali concentration to produce a viscose having a composition of 7.5% cellulose and 5.7% total alkalinity. During the dissolving process the methyl chloride quaternary derivative of an ethoxylated quaternary ammonium compound having the general formula:



35 wherein  $x+y=$  approximately 15 ethylene oxide units and  $\text{R}$  is a saturated straight chain hydrocarbon radical containing 8-18 carbon atoms in the amount of 1.0% (C.I.V.) and polymerized ethylene oxide having an average molecular weight of about 4000 in the amount of 1.0% (C.I.V.) were added.

30 The viscose containing the just mentioned combination of additives was permitted to age to a maturity value of 14-16 NH<sub>4</sub>Cl number. After conventional filtering and deaerating, the viscose was formed into a thread of 1650 denier, 720 filament viscose rayon yarn by extrusion of the viscose through a spinneret into an aqueous coagulating bath having a temperature of 65° C. and containing 4.8% H<sub>2</sub>SO<sub>4</sub>, 12% Na<sub>2</sub>SO<sub>4</sub> and 3.5% ZnSO<sub>4</sub>.

45 After being passed through the coagulating bath, the thread was withdrawn therefrom by means of a first godet. Then the thread was guided into and through a second hot weakly acidic bath at a temperature of 94° C. and withdrawn therefrom by means of a second godet. Due to a predetermined differential in the peripheral speeds of said godets, the thread was stretched 50 98% therebetween. The yarn draw off speed was 55 meters per minute. The aftertreatment of the thread 55 was carried out according to the usual processes which includes drying of the thread. Then the thread was given a slashing stretch of about 12% and thereafter dried 60 under tension. The slashed thread was twisted and plied into the tire cord construction of 11.4 x 10.6.

65 For comparison purposes, threads were produced under the same conditions mentioned above in this example except that the sole additive employed was the polyethylene oxide compound of the present example in the amount of 2.0% (C.I.V.). Moreover, threads were also produced under these conditions but while using only the quaternary amine additive of the present example in the amount of 2.5% (C.I.V.).

70 The strength properties of the threads so produced are listed in Table I for comparison, from which it is seen that according to the present invention there is a significant increase in both the conditioned and oven dry cord 75 properties.

5  
Table I

| Strength, g./100 den.             | Quaternary amine + polyethylene oxide | Quaternary amine only | Polyethylene oxide only |
|-----------------------------------|---------------------------------------|-----------------------|-------------------------|
| Slashed singles, conditioned..... | 443                                   | 437                   | 440                     |
| Slashed singles, wet.....         | 316                                   | 313                   | 307                     |
| Cord, conditioned.....            | 379                                   | 355                   | 345                     |
| Cord, oven dry.....               | 449                                   | 433                   | 406                     |

## EXAMPLE II

A viscose having a composition of 7.5% cellulose and 5.5% total alkalinity was prepared in the manner described in Example I. To this viscose the ethoxylated quaternary amine and the polyethylene oxide additives used in Example I were added in the amounts of 2.0% (C.I.V.) and 1.0% (C.I.V.), respectively. After aging, filtering and deaerating, the viscose was formed into a thread of 1650 denier, 720 filament viscose rayon yarn by extrusion through a spinneret into an aqueous acidic coagulating bath having a temperature of 51° C. and containing 5.2% H<sub>2</sub>SO<sub>4</sub>, 12% Na<sub>2</sub>SO<sub>4</sub> and 5.0% ZnSO<sub>4</sub>.

After being passed through the coagulating bath, the thread was withdrawn therefrom by means of a first godet. Then, the thread was guided into and through a second hot weakly acidic bath at a temperature of 94° C. and withdrawn therefrom by means of a second godet. Due to a predetermined differential in the peripheral speeds of said godets, the thread was stretched 100% therebetween. The yarn draw-off speed was 65 meters per minute. The aftertreating of the thread was carried out according to the usual processes. Then the thread was given a slashing stretch of about 12% and thereafter dried under tension. The slashed thread was plied into the tire cord construction of 12.0 x 12.0.

For comparison purposes, threads were produced under the same conditions mentioned above in this example except that the sole additive employed was the polyethylene oxide compound of the present example in the amount of 2.0% (C.I.V.). Moreover, threads were also produced under these conditions while using only the quaternary amine additive of the present example in the amount of 2.7% (C.I.V.).

The strength properties of the threads so produced are listed in Table II for comparison, from which it is seen that according to the present invention there is a significant increase in both the conditioned and oven dry cord properties.

Table II

| Strength, g./100 den.               | Quaternary amine + polyethylene oxide | Quaternary amine only | Polyethylene oxide only |
|-------------------------------------|---------------------------------------|-----------------------|-------------------------|
| Unslashed singles, conditioned..... | 461                                   | 434                   | 453                     |
| Slashed singles, conditioned.....   | 442                                   | 450                   | .....                   |
| Slashed singles, wet.....           | 321                                   | 317                   | .....                   |
| Cords, conditioned.....             | 350                                   | 338                   | 339                     |
| Cords, oven dry.....                | 422                                   | 400                   | 378                     |

## EXAMPLE III

A viscose having a composition of 7.5% cellulose and 5.7% total alkalinity was prepared in the manner described in Example I. The viscose after being properly filtered, deaerated and aged was pumped to a spinneret through a conduit. A solution containing the combination of additives used in Example I was injected and later intimately mixed in the amounts of 1.5% (C.I.V.) ethoxylated quaternary amine and 1.0% (C.I.V.) polyethylene oxide into the viscose in the manner described in copending application Serial No. 655,004, filed April 25, 1957, and having common ownership herewith.

The viscose containing the additives was formed into a thread of 1650 denier, 1100 filament viscose rayon yarn

## 6

in an aqueous acidic coagulating bath having a temperature of 55° C. and containing 4.7% H<sub>2</sub>SO<sub>4</sub>, 12% Na<sub>2</sub>SO<sub>4</sub> and 4.4% ZnSO<sub>4</sub>. The freshly spun thread was stretched 93%, aftertreated and slash stretched as described in Example II. The thread was then plied into the tire cord construction of 11.4 x 10.6.

For comparison purposes, threads were produced under the same conditions mentioned above in this example except that the sole additive employed was the polyethylene oxide compound of the present example in the amount of 2.0% (C.I.V.). Moreover, threads were also produced under these conditions while using only the quaternary amine additive of the present example in the amount of 2.0% (C.I.V.).

The strength properties of the threads so produced are listed in Table III for comparison from which it is seen that there is a significant increase in conditioned and oven dry cord properties and in wet slashed singles strength.

20

Table III

| Strength, g./100 den.               | Quaternary amine + polyethylene oxide | Quaternary amine only | Polyethylene oxide only |
|-------------------------------------|---------------------------------------|-----------------------|-------------------------|
| 25                                  |                                       |                       |                         |
| Unslashed singles, conditioned..... | 445                                   | 448                   | 436                     |
| Slashed singles, conditioned.....   | 502                                   | 504                   | 492                     |
| Slashed singles, wet.....           | 366                                   | 358                   | 313                     |
| Cords, conditioned.....             | 422                                   | 420                   | 382                     |
| Cords, oven dry.....                | 494                                   | 481                   | 447                     |
| 30                                  |                                       |                       |                         |

## EXAMPLE IV

A viscose having a composition of 7.5% cellulose and 5.6% total alkalinity was prepared in the manner described in Example I. To this viscose the ethoxylated quaternary amine and the polyethylene oxide additives used in Example I were added in the amounts of 1.5% (C.I.V.) and 0.5% (C.I.V.), respectively. After aging, filtering and deaerating, the viscose was formed into a thread of 1100 denier, 720 filament in an aqueous acidic coagulating bath having a temperature of 55° C. and containing 4.6% H<sub>2</sub>SO<sub>4</sub>, 12% Na<sub>2</sub>SO<sub>4</sub> and 4.4% ZnSO<sub>4</sub>. The freshly spun thread was stretched 98%, aftertreated and slash stretched as described in Example II. The thread was then plied into the tire cord construction of 14.0 x 11.5.

For comparison purposes, threads were produced under the same conditions mentioned above in this example except that the sole additive employed was the quaternary amine additive of the present example in the amount of 2.5% (C.I.V.).

The strength properties of the threads so produced are listed in Table IV for comparison from which it is seen that there is a significant increase in conditioned and oven dry cord properties.

Table IV

| Strength, g./100 den.               | Quaternary amine + polyethylene oxide | Quaternary amine only |
|-------------------------------------|---------------------------------------|-----------------------|
| 60                                  |                                       |                       |
| Unslashed singles, conditioned..... | 444                                   | 425                   |
| Slashed singles, conditioned.....   | 483                                   | 465                   |
| Slashed singles, wet.....           | 343                                   | 320                   |
| Cords, conditioned.....             | 422                                   | 384                   |
| Cords, oven dry.....                | 515                                   | 451                   |
| 65                                  |                                       |                       |

## EXAMPLE V

A viscose having the composition of 7.5% cellulose and 5.6% total alkalinity was prepared in the manner described in Example I. Polymerized ethylene oxide having an average molecular weight of 2000 in the amount of 1.5% (C.I.V.) and the ethoxylated quaternary amine used in Example I in the amount of 0.5% (C.I.V.) were added to a portion of the viscose. To another portion

75

of the viscose polymerized ethylene oxide having an average molecular weight of 1000 in the amount of 1.0% (C.I.V.) and the ethoxylated quaternary amine used in Example I in the amount of 1.0% (C.I.V.) were added. To a third portion of the viscose polymerized ethylene oxide having an average molecular weight of 1000 in the amount of 2.5% (C.I.V.) was added.

These viscoses were produced into threads in a manner identical to Example IV. The strength values of these threads are reported in Table V from which it is seen that the tenacities of the threads produced using polyethylene oxide having the lower molecular weight of 1000, either alone or together with the quaternary amine were considerably lower as compared to the tenacities of the thread produced under the influence of both the polyethylene oxide compound having the molecular weight of 2000 and the quaternary amine in accordance with the present invention.

Table V

| Strength, g./100 den.                  | 1.5% (C.I.V.)<br>Polyethylene<br>oxide (M.W. =<br>2,000)+0.5%<br>(C.I.V.)<br>quaternary<br>amine | 1.0% (C.I.V.)<br>Polyethylene<br>oxide (M.W. =<br>1,000)+1.0%<br>(C.I.V.)<br>quaternary<br>amine | 2.5% (C.I.V.)<br>Polyethylene<br>oxide (M.W. =<br>1,000) only |
|----------------------------------------|--------------------------------------------------------------------------------------------------|--------------------------------------------------------------------------------------------------|---------------------------------------------------------------|
| Unslashed singles,<br>conditioned..... | 463                                                                                              | 470                                                                                              | 458                                                           |
| Slashed singles, con-<br>ditioned..... | 504                                                                                              | 486                                                                                              | 485                                                           |
| Slashed singles, wet.....              | 347                                                                                              | 338                                                                                              | 331                                                           |
| Cords, conditioned.....                | 415                                                                                              | 395                                                                                              | 395                                                           |
| Cords, oven dry.....                   | 494                                                                                              | 484                                                                                              | 471                                                           |

While preferred embodiments of the invention have been shown, it is to be understood that changes and variations may be made without departing from the spirit and scope of the invention so defined by the appended claims.

What is claimed is:

1. A method of producing viscose rayon filaments having improved strength comprising spinning a thread from a viscose containing a compound having the general formula:



where R is an alkyl radical with at least 6 carbon atoms;  $x+y=2-50$  and Z is an innocuous anion, in the amount of 0.5 to 5.0% by weight based on the cellulose content and polyethylene oxide having a molecular weight in the range of 1500-4500 in the amount of 0.5 to 5.0% by weight based on the cellulose content, the total minimum amount of said compound and polyethylene oxide being at least 2.0% by weight based on the cellulose content, into an aqueous spinbath containing less than 7% sulfuric acid and at least 2% zinc sulfate and stretching the freshly spun thread.

2. A method of producing viscose rayon filaments having improved strength comprising adding to a viscose the methyl chloride quaternary derivative of an ethoxylated quaternary ammonium compound, having the general formula:



- 5 wherein  $x+y=$  approximately 15 and R is a saturated, straight chain, hydrocarbon radical containing 8-18 carbon atoms in the amount of about 1-2% by weight based on the cellulose content and polyethylene oxide having a molecular weight in the range of 1500-4500 in the amount of about 0.5-1.0% by weight based on the cellulose content, the total minimum amount of said compound and polyethylene oxide being at least 2.0% by weight based on the cellulose content, spinning the resulting viscose into a thread in an aqueous coagulating bath containing less than 7% sulfuric acid and at least 2% zinc sulfate, and passing the freshly spun thread into a second weakly acidic bath at a temperature above 80° C. while stretching the thread to the extent of at least 80%.

3. A viscose spinning composition containing a compound having the general formula:



- 25 where R is an alkyl radical with at least 6 carbon atoms;  $x+y=2-50$  and Z is an innocuous anion, in the amount of 0.5 to 5.0% by weight based on the cellulose content and polyethylene oxide having a molecular weight in the range of 1500-4500 in the amount of 0.5-5.0% by weight based on the cellulose content, the total minimum amount of said compound and polyethylene oxide being at least 2.0% by weight based on the cellulose content.

4. A viscose spinning composition containing an ethoxylated quaternary ammonium compound, having the general formula:



- 40 where  $x+y=$  approximately 15 and R is a saturated, straight chain, hydrocarbon radical containing 8-18 carbon atoms in the amount of about 1-2% by weight based on the cellulose content and polyethylene oxide having a molecular weight in the range of 1500-4500 in the amount of about 0.5-1.0% by weight based on the cellulose content, the total minimum amount of said compound and polyethylene oxide being at least 2.0% by weight based on the cellulose content.

50

#### References Cited in the file of this patent

#### UNITED STATES PATENTS

- |           |                 |                |
|-----------|-----------------|----------------|
| 2,572,217 | Thurmond        | Oct. 23, 1951  |
| 2,593,466 | MacLaurin       | Apr. 22, 1952  |
| 2,648,611 | Richter         | Aug. 11, 1953  |
| 2,696,423 | Dietrich        | Dec. 7, 1954   |
| 2,705,184 | Drisch          | Mar. 29, 1955  |
| 2,732,279 | Tachikawa       | Jan. 24, 1956  |
| 2,759,975 | Chiddix         | Aug. 21, 1956  |
| 2,852,334 | Hollihan        | Sept. 16, 1958 |
| 2,860,480 | Cox             | Nov. 18, 1958  |
| 2,937,922 | Mitchell et al. | May 24, 1960   |